

June 16, 1959

W. L. ARNOLD ET AL

2,890,971

COATING METHOD

Filed May 2, 1956



INVENTORS  
WALTER L. ARNOLD  
ROBERT K. PEARCE

BY  
William A. Zelask  
ATTORNEY

1

2,890,971

## COATING METHOD

Walter L. Arnold, New Providence, and Robert K. Pearce, Maplewood, N.J., assignors to Radio Corporation of America, a corporation of Delaware

Application May 2, 1956, Serial No. 582,243

9 Claims. (Cl. 117—65)

This invention relates to a coating method, and in particular to a method of coating articles with a refractory insulating material such as, for example, aluminum oxide. The method of the invention is particularly advantageous in coating a metallic base in wire or ribbon form with aluminum oxide to make heaters for indirectly heated electron tube cathodes.

One of the common types of heaters for indirectly heated cathodes comprises a tungsten wire coated with aluminum oxide, the oxide coating forming an insulating covering for the heater so that when the heater is inserted into a cathode sleeve the heater and sleeve are insulated from each other. Consequently, it is desirable to provide the heater with a strongly adherent coating to prevent the coating from being stripped from the metallic base of the heater during normal handling. However, the ends of the heater must be bared in order that the metallic base of the heater be exposed for welding to lead-in wires. Consequently, the coating must also be soft enough so that it can be easily chipped or broken away from the metallic base at the places to be bared. In addition, the portions of the base so bared must be relatively free of oxidation so that they may be in a proper condition for welding.

It is therefore an object of the invention to provide an improved method for making a coated heater having an insulating coating, such as aluminum oxide, which is relatively strongly adherent to its base material and which at the same time has bared base material portions adapted to be welded to lead-in wires.

It is another object of the invention to provide an improved method of coating a metallic base and wherein the hardness of the coating is controllable without oxidizing the base.

The foregoing and related objects are achieved in a method wherein a base to be coated is first subjected to one or more coating steps. Each coating step includes the passing of the base through a mixture including aluminum oxide and a binder, followed by a drying of the coated base in air at a temperature high enough to dry the coating but insufficient to oxidize the coated base. Then the base thus coated is immersed in a bath containing aluminum nitrate of a predetermined concentration. Finally, the coated base is subjected to heat in a reducing atmosphere, as by being passed through a hydrogen furnace. The stock thus made has an insulating coating which is hard enough to withstand normal handling and which may be selectively, relatively easily removed, as by a chipping or cracking of the coating.

One example of a method of the invention involves a heater wire comprised of a metallic base, which may be tungsten, to which an aluminum oxide coating is applied. As indicated in the sole figure of the drawing, the first operation is to coat a bare metallic wire with wetted aluminum oxide. A preferred method of applying this aluminum oxide coating is to pass the wire through a slurry containing aluminum oxide and a binder in a liquid vehicle then to dry the coating thus produced in an air

2

oven. The desired thickness of aluminum oxide coating is achieved by passing the wire successively through the slurry and the air oven through a number of cycles until the desired coating thickness is built up on the wire. For example, if a bare tungsten wire 1.24 mils in diameter is to be coated with aluminum oxide to a coating thickness of 5 mils, about 12 passes of the wire through the slurry and oven are usually required.

As a relatively hard coating of aluminum oxide is desired, the temperature of the air oven in the above drying step has, in the prior art, usually been from about 680° C. to about 800° C. However, a heating to such a temperature causes the base material of the wire, in this case tungsten, to oxidize. The oxide layer thus formed cannot be practicably removed in order to carry out a desired welding step. It has been found that the maximum temperature to which the aluminum oxide coated wire can be subjected, during an air drying operation, without forming an oxide layer which cannot be practicably removed, is a temperature of about 600° C., and preferably a temperature of not exceeding 550° C. However, when a temperature of less than about 680° C. is used to dry the aluminum oxide coating as it is formed, the coating is too soft to withstand the handling operations encountered before the wire is mounted within a cathode sleeve.

The invention provides a means for overcoming the above-described problem of excessive oxidation at the temperature required to provide the desired coating hardness in the air drying steps.

As indicated in the drawing, it has been found that the additional steps of immersing the aluminum oxide coated wire in a bath containing aluminum nitrate, followed by a passage of the wire through a reducing furnace, hardens a coated wire which has been subjected to an air drying step at a temperature of less than 600° C. and also substantially removes any residual oxide layer which may have formed in any of the preceding steps.

A preferred aluminum oxide coating slurry used in practicing the invention is comprised of the following. To make a half gallon slurry, mix 360 cc. methyl alcohol and 285 grams of 900 mesh aluminum oxide powder. This mixture is ball milled for about three hours. This ball milling operation appears to break up any agglomerates which are present in the 900 mesh powder. After the ball milling there is added to the milled mixture 2,625 grams of 500 mesh aluminum oxide powder, 326 cc. of distilled water, and 490 cc. of a saturated solution of aluminum nitrate in water for service as a binder.

A tungsten wire is passed through the slurry above described and then passed through an air oven heated to a temperature of between from about 500° C. to about 600° C. At any event the temperature should not exceed 600° C. else an oxide layer will be formed which cannot be readily removed by later operations. A preferred temperature is about 550° C., a lower temperature giving a softer coating and a higher temperature giving a harder coating. The wire is passed through the slurry and air oven in a sufficient number of cycles to build up the coating to the desired thickness. Then the coated wire is immersed in a bath containing aluminum nitrate in water. The aluminum nitrate concentration is preferably from about 30 percent to about 100 percent of a saturated solution (at ordinary room temperatures) to impart a substantial increase in the hardness of the coating. While the exact concentration of aluminum nitrate is not critical, the concentration should be relatively high to assure the pick up of sufficient nitrate to increase the hardness of the coating to the desired extent. For example, a preferred bath consists of a substantially completely saturated solution of aluminum nitrate at ordinary room temperatures.

The wire is then passed through a reducing furnace at a temperature of between about 800° C. and 1000° C. The wire remains in this furnace for a length of time sufficient to dry it. The atmosphere of the reducing furnace is preferably one which consists essentially of hydrogen. The hardness of the coating is softened by increasing oven temperatures. (This softening with increasing temperatures holds true up to sintering temperature, that is, roughly about 1550° C.). When the wire has been subjected to an air oven temperature of about 550° C., and to an aluminum nitrate bath comprised of a substantially saturated solution of aluminum nitrate in water, the desired reducing furnace temperature is about 1000° C. This provides a coating having a desired hardness for good adherence of the coating and at the same time permits easy removal of the coating at the portions to be involved in welds. The passage of the wire through the reducing furnace, however, does not affect the hardness of the coating as much as the air oven heating and the aluminum nitrate bath. Consequently, the greatest amount of control over the coating hardness can be exercised by a control of the air oven temperature and of the concentration of the aluminum nitrate in the bath.

The wire produced by the aforescribed steps is then wound into heater form and finally cut off to desired lengths for use as heaters in electron tubes. The portions of the wire which are to be welded to lead-in wires are subjected to any of the well known chipping or cracking operations which break off the coating only at these wire portions.

It will be noted that up to this point the wire has not been subjected to a temperature as high as sintering temperature. However, after the heater is mounted within an electron tube, and during the usual bake-out and evacuation step in the manufacture of the tube, the heater is subjected to a temperature at least as high as the sintering point (at least about 1550° C.) of the coating. This last heating sinters the aluminum oxide of the coating and rids the coating of substantially all other matter.

It is seen from the foregoing that the method of the invention provides a means for controlling the hardness of an aluminum oxide coating on a metallic base. The hardness of the coating may be controlled by adjusting the temperature of the air oven, by adjusting the concentration of the aluminum nitrate in the aluminum nitrate bath, or by adjusting the temperature of the reducing furnace. The method of the invention thus provides a means for making improved cathode heaters having an insulating coating which is relatively strongly adherent to the base material and which at the same time has bared base material portions adapted to be welded to lead-in wires.

What is claimed is:

1. A coating method comprising the steps of successively coating an oxidizable metallic base with a mixture including aluminum oxide and an aluminum nitrate binder to form a coating on said base, drying in air the coating thus formed at a temperature high enough to dry the coating but insufficient to oxidize the coated base to a degree wherein the oxide resists chemical removal, whereby the coating is relatively soft, then immersing the coated base in a bath consisting essentially of aluminum nitrate and a solvent for said nitrate, and then heating the coated base in a reducing atmosphere to a temperature of from about 800° C. to about 1000° C. for simultaneously increasing the hardness of the coating for substantially easy removal of selected portions thereof, and removing chemically any oxide formed on said base during said air drying.

2. A coating method comprising the steps of successively coating a metallic base with a mixture including aluminum oxide and an aluminum oxide binder to pro-

vide a coating on said base, drying said coating in air heated to a temperature between room temperature and about 600° C., whereby said coating acquires a first and relatively low order of hardness and a chemically removable oxide is formed on said base, immersing the coated base in a bath consisting essentially of aluminum nitrate and a solvent for said nitrate, and then heating the coated base in a reducing atmosphere at a temperature higher than about 600° C. and up to 1000° C. for simultaneously removing said oxide and imparting a second and relatively high order of hardness to said coating, whereby a metallic base is provided which is substantially oxide-free, and which has an aluminum oxide coating which is relatively strongly adherent to said base and which is adapted to be selectively, relatively easily removed therefrom.

3. A coating method comprising the steps of successively coating a metallic base with a mixture including aluminum oxide and an aluminum nitrate binder, drying the coated base thus formed in hot air, at a temperature high enough to dry the coating but insufficient to oxidize the coated base, immersing the coated base in a bath consisting essentially of aluminum nitrate and a solvent for said nitrate, and then heating the coated base to a temperature of from about 800° C. to about 1000° C. in a reducing atmosphere consisting essentially of hydrogen, whereby a metallic base is provided which is substantially oxide-free, and which has an aluminum oxide coating which is relatively strongly adherent to said base and which is adapted to be selectively, relatively easily removed therefrom.

4. A coating method comprising the steps of successively coating a tungsten base with a mixture including aluminum oxide and an aluminum nitrate binder, drying the coated base thus formed in air heated to a temperature of between about 500° C. and about 600° C., immersing the coated base in a bath consisting essentially of aluminum nitrate and a solvent for said nitrate, and then heating the coated base to a temperature of between about 800° C. and about 1000° C. in a substantially dry hydrogen atmosphere, whereby a tungsten base is provided which is substantially oxide free, and which has an aluminum oxide coating which is relatively strongly adherent to said base and which is adapted to be selectively, relatively easily removed therefrom.

5. A coating method comprising the steps of successively coating a tungsten base with a mixture including aluminum oxide and an aluminum nitrate binder, drying the coated base thus formed in an air oven at a temperature of between about 500° C. and about 600° C., immersing the coated base in a bath consisting essentially of a substantially saturated solution of aluminum nitrate in water, and then heating the coated base to a temperature of between about 800° C. and about 1000° C. in a substantially dry hydrogen atmosphere, whereby a tungsten base is provided which is substantially oxide free, and which has an aluminum oxide coating which is relatively strongly adherent to said base and which is adapted to be selectively, relatively easily removed therefrom.

6. A coating method comprising the steps of successively coating a tungsten base with a mixture including aluminum oxide and a saturated aqueous solution of aluminum nitrate, drying the coated base thus formed in an air oven at a temperature of between about 500° C. and about 500° C., immersing the coated base in a bath consisting essentially of aluminum nitrate and a solvent for said nitrate, and then heating the coated base to a temperature of between about 800° C. and about 1000° C. in a substantially dry hydrogen atmosphere for a period of time sufficient to reduce the base material to substantially oxide-free tungsten, whereby a tungsten base is provided which is substantially oxide free, and which has an aluminum oxide coating which is relatively strong-

ly adherent to said base and which is adapted to be selectively, relatively easily removed therefrom.

7. A coating method comprising the steps of first coating a metallic base by subjecting said base to a plurality of operations each comprising a pass through a slurry of aluminum oxide in an aqueous solution of aluminum nitrate followed by a drying of the base in air heated to a temperature of between about 500° C. and about 600° C., then immersing the base thus coated in a bath consisting essentially of a 30 to 100 percent saturated solution at ordinary room temperatures of aluminum nitrate in water, and finally heating the base to a temperature of between about 800° C. and about 1000° C. in substantially dry atmosphere consisting essentially of hydrogen and for a period of time sufficient to reduce the base material to a substantially oxide free form, whereby a metallic base is provided which is substantially oxide free, and which has an aluminum oxide coating which is relatively strongly adherent to said base and which is adapted to be selectively, relatively easily removed from said base.

8. A coating method comprising the steps of first coating a metallic base by subjecting said base to a plurality of operations each comprising a pass through a slurry of aluminum oxide in an aqueous solution of aluminum

5

10

15

20

nitrate followed by a drying of the base in an air oven at a temperature of about 550° C., then subjecting the base thus coated to a bath consisting essentially of a substantially saturated solution at ordinary room temperatures of aluminum nitrate in water, and finally subjecting the base to heat at a temperature of about 1000° C. in a substantially dry atmosphere consisting essentially of hydrogen and for a period of time sufficient to reduce the base material to a substantially oxide free form, whereby a metallic base is provided which is substantially oxide free, and which has an aluminum oxide coating which is relatively strongly adherent to said base and which is adapted to be selectively, relatively easily removed from said base.

9. The product of the process of claim 1.

References Cited in the file of this patent

UNITED STATES PATENTS

|           |           |               |
|-----------|-----------|---------------|
| 2,008,733 | Tosterud  | July 23, 1955 |
| 2,043,720 | Wagenhals | June 9, 1936  |
| 2,179,453 | Palmateer | Nov. 7, 1939  |
| 2,722,491 | Anderson  | Nov. 1, 1955  |
| 2,743,192 | White     | Apr. 24, 1956 |

UNITED STATES PATENT OFFICE  
CERTIFICATE OF CORRECTION

Patent No. 2,890,971

June 16, 1959

Walter L. Arnold et al.

It is hereby certified that error appears in the printed specification of the above numbered patent requiring correction and that the said Letters Patent should read as corrected below.

Column 4, lines 66 and 67, for "about 500° C. and about 500° C."  
read -- about 500° C. and about 600° C. --.

Signed and sealed this 23rd day of February 1960.

(SEAL)  
Attest:

KARL H. AXLINE  
Attesting Officer

ROBERT C. WATSON  
Commissioner of Patents